

E. E. NOVOTNY.  
COMPOSITE SHEET.  
APPLICATION FILED MAY 20, 1916.

1,377,502.

Patented May 10, 1921.

*Fig. 1,*



*Fig. 2,*



Inventor

Emil E. Novotny  
By his Attorney.

Meyers, Bushman & Rea

# UNITED STATES PATENT OFFICE.

EMIL E. NOVOTNY, OF RIVERSIDE, ILLINOIS, ASSIGNOR TO J. STOGDELL STOKES, OF MOORESTOWN, NEW JERSEY.

## COMPOSITE SHEET.

1,377,502.

Specification of Letters Patent. Patented May 10, 1921.

Application filed May 20, 1916. Serial No. 98,909.

To all whom it may concern:

Be it known that I, EMIL E. NOVOTNY, a citizen of the United States, residing at Riverside, in the county of Cook and State of Illinois, have invented certain new and useful Improvements in Composite Sheets, of which the following is a specification.

The present invention relates to a composition sheet for making matrices or molds, and has particular application to a sheet adapted for making a matrix or mold to be used in the manufacture of printing plates.

As is well known to those in the printing art, printing plates are comparatively expensive because they require special appliances and the exercise of considerable skill in their manufacture, and therefore, when a printer desires to have a body of type or a cut or relief plate reproduced as a printing plate it is necessary for him to have this work done in an establishment usually making a specialty of this particular line of work.

In the present instance it is my purpose to provide a sheet which is particularly well adapted for making printing plates and which can be sold to the printer in quantity at a relatively low cost, so that by a simple method, such, for instance, as is described in my co-pending application Serial No. 98,910, filed May 20, 1916, he can make his own mold in his own establishment, and can then make his own printing plates from such mold.

With the above recited objects and others of a similar nature in view, the invention consists in the improved composite sheet and in the method of making the same set forth in and falling within the scope of the appended claims.

In the accompanying drawings:

Figure 1 is perspective view of one form of my mold sheet.

Fig. 2 is a cross sectional view taken through the same.

In the practice of the invention I select a thin sheet or layer of metal preferably possessing a certain degree of pliability and capable of being rendered plastic, but having comparatively little ductility, the preferable metal employed being lead, although other metals, such as copper, may be used. One face of this lead sheet, that is, the face which will constitute the back of the mold sheet is preferably electro-plated with cop-

per. To this back face of the lead sheet I apply, in any suitable manner, a selected cement-like substance, when the latter is in a plastic condition, this substance being such that when in its hardened or non-plastic state it will not lose its form. There are various kinds of cements and embossing compositions which I might employ to form this backing sheet or layer, which is shown at B, but I have found that a plastic phenolic condensation product which as is well known is a synthetic resin or resinous composition capable of being hardened to the infusible or non-plastic state and which will not leave this form when it sets is admirable for this purpose. There are several kinds or varieties of these phenolic condensation products well known in the art to which they relate, one of which is known as "bakelite" and is well adapted for my purpose. This cement is applied in its plastic state to the back of the lead sheet A to form a backing coating, layer or sheet of a suitable thickness, for instance, about twenty one-thousandths of an inch. While this cement is still in a plastic or pliable state or condition I preferably place an outer backing sheet or layer thereon, shown at C and which backing sheet is preferably in the nature of flexible, fibrous material such as paper-board. This backing sheet C is employed for the sake of economy in the use of cement and also to facilitate the molding operation, for if desired, instead of employing this paper-board backing sheet C, which is of substantially the same thickness as the layer or cement sheet B, I may increase the thickness of the cement layer or sheet B, and dispense with the paper-board sheet C, so that my composite plate in such case would be composed of a metallic facing sheet and a cementitious backing sheet. The purpose of employing the cement backing sheet B is to provide a yieldable backing for the lead facing sheet which backing will be yielding and resilient under pressure in making the mold or matrix and will also provide a neutral point for the flow of the lead material in bending a matrix or mold made from the sheet, for the purpose of forming a curved or bowed mold for the manufacture of curved or partly cylindrical printing plates.

It is of course to be understood that the various sheets or layers going to make up

this composite plate may be of any desired thickness, and that as many layers or sheets as may be deemed necessary in the use of a particular composite plate may be employed.

- 5 In order to increase the adherence of the cementitious sheet to the lead sheet and to thereby avoid the peeling of such cementitious sheet from the back of the lead sheet I coat the back face of the lead sheet by electroplating with copper, tin or the like, thereby insuring coherence between the sheets, because of the fact that the film produced by the electroplating will possess a certain degree of porosity, and will therefore act as 10 a binder to anchor or hold the cementitious sheet to the lead sheet.

While I have herein shown and described one particular embodiment of my invention I wish it to be understood that I do not confine myself to all the precise details of con- 15

struction herein set forth by way of illustration as modification and variation may be made without departing from the spirit of the invention or exceeding the scope of the appended claims.

What I claim is:

1. A composite sheet comprising a metallic facing sheet, and a cementitious backing sheet capable of assuming a hard, set and infusible form under heat and pressure, 30 said facing sheet having its back provided with a porous coating to insure coherence of the two sheets.

2. A composite sheet comprising a metallic facing sheet and a hard, cementitious 35 backing sheet, said facing sheet having its back provided with an electro-plated coating to insure coherence of the two sheets.

In testimony whereof I affix my signature.

EMIL E. NOVOTNY.